

## UNITED STATES PATENT OFFICE

2,221,184

## PRODUCTION OF TEXTILE MATERIALS

George Holland Ellis and Robert Wighton Moncrieff, Spondon, near Derby, England, assignors to Celanese Corporation of America, a corporation of Delaware

No Drawing. Application October 22, 1938, Serial No. 236,576. In Great Britain November 10, 1937

2 Claims. (Cl. 8—121)

This invention relates to improvements in or relating to the production of textile materials, and particularly to a process for modifying the affinity of cellulosic textile materials for cotton

5 colours.

It is well-known that various types of natural and artificial cellulosic materials may be employed in the manufacture of fabrics, articles of clothing and other goods, examples of such 10 materials being cotton, linen and regenerated cellulose materials obtained by the viscose, cuprammonium and nitrocellulose processes and by the saponification of textile materials made of cellulose acetate or other organic esters of cellulose. While all these cellulosic materials have an 15 affinity for cotton dyestuffs, the degree of affinity of one type of material may differ from that of another type of material, and indeed the degree of affinity of the same type of material may vary 20 according to the processes to which it has been subjected. Thus, for example, the degree of affinity of mercerised cotton may be different from that of unmercerised cotton, and that of artificial cellulosic materials obtained by the 25 saponification of ordinary dry spun cellulose acetate yarn may be different from that of such materials obtained by the saponification of stretched cellulose acetate yarn.

In consequence of the different affinities of the 30 various types of cellulosic materials, difficulty may arise when it is desired to colour articles containing two or more types of cellulosic materials in a solid shade as, for example, in the dyeing of hose, in which the tops and feet are 35 frequently of cotton and the legs of regenerated cellulose yarn.

It has now been discovered that the dyeing difficulties referred to above may be avoided by 40 subjecting the materials having the greater affinity for cotton dyestuffs to an esterification or etherification process, so as to introduce a small proportion of organic radicle into the materials. In general, when only two types of cellulosic materials are to be employed in the production of 45 an article it is necessary to esterify or etherify only the constituent which has the greater affinity for the cotton dyestuff. Thus, for example, in general cotton has a greater affinity for cotton dyestuffs than has regenerated cellulose yarn obtained by the saponification of stretched cellulose 50 acetate yarn, and in such a case the cotton yarn is slightly esterified or etherified. On the other hand, regenerated cellulose yarn obtained by the viscose and cuprammonium processes usually has more affinity for cotton dyestuffs than

has cotton yarn, so that when these types of materials are to be combined in the production of an article it is the regenerated cellulose yarn which is esterified or etherified. The exact degree of esterification or etherification of course 5 depends upon the particular circumstances, especially upon the two types of materials which are to be combined, but in general the degree of esterification or etherification necessary corresponds to a weight increase of 5% or less, particularly about 1.5 to 2.5%.

The invention includes the process of modifying the affinity of cellulosic yarn, the production of fabrics and other materials containing purely 15 cellulosic yarns and the modified yarns, and the process of colouring the fabrics and other materials in solid shades with cotton dyestuffs.

The most suitable agent for treatment of the materials is acetic anhydride, though other esterifying agents, for example acetyl chloride, propionic and butyric anhydrides and other lower fatty acid derivatives, i. e. of an acid containing not more than six carbon atoms may, if desired, be employed. Etherifying agents, e. g. ethyl chloride and dimethyl sulphate, may also be used. 20 The treatment is carried out under such conditions that the structure of the materials is not changed, and it is usually desirable to effect it in the presence of a liquid diluent which is a non-solvent for the materials and solvent for the 25 esterifying or etherifying agent employed. When esterification is effected with an acid anhydride suitable catalysts may be employed, examples of which are ferric, stannic and zinc chlorides, preferably used in conjunction with hydrochloric acid 30 or a small proportion of acid chloride. Acid catalysts such as sulphuric acid or perchloric acid 35 may be used, but they are in general less suitable, and if employed should be used at low temperatures and in a low concentration. If acid chlorides or alkyl halides or sulphates are employed, preferably a small proportion of basic substance, which may be organic or inorganic, is present to neutralise the acid formed during the 40 reaction.

The following is an example of the treatment of cotton according to the process of the present invention in order to reduce slightly its affinity for cotton dyestuffs:

Cotton yarn in hank form is first boiled for 50 about 4-6 hours in a 1% solution of caustic soda at a temperature of 120 to 130° C. and washed off well. It is then treated for 20 to 30 minutes at about 30° C. in a 1% solution of sodium hypochlorite. The hanks are then drained, treated

in a .5% solution of acetic acid for 15 to 30 minutes at about 20° C., washed off well and next treated for about 10 minutes at 20° C. in an anti-chlor bath consisting of a .2% solution of sodium sulphite. They are then well washed off, dried and pretreated in 96% acetic acid for about 15 minutes at 20 to 25° C., washed off with acetone and drained. They are then treated for 15 minutes at about 20° C. in a bath having the following 10 ing composition, the bath ratio being about 40:1.

|                      | Parts |
|----------------------|-------|
| Carbon tetrachloride | 57.5  |
| Acetic anhydride     | 30    |
| 15 Acetic acid       | 11.5  |
| Acetyl chloride      | 1     |
| Zinc chloride        | 1     |

After completion of the treatment the yarn is removed from the bath, washed off with carbon tetrachloride and air-dried. Finally, it is washed off in 5% acetic acid followed by a weak ammonia bath and dried.

The invention includes all kinds of mixed textile materials containing purely cellulosic yarns and the modified yarns. Thus, for example, the two types of yarns may be present in doubled yarns or in a woven, knitted or netted fabric. In the case of woven fabrics the weft may consist wholly of one type of yarn and the warp wholly of the other type of yarn or both types of yarn may be in the weft and/or in the warp.

The mixed textile materials may be dyed with any suitable cotton dyestuffs but it will be understood that the particular dyestuff employed will 35 depend to some extent on the proportion and

nature of the organic substituent radicle present in the modified textile material. Examples of dyestuffs which may be employed are Chrysamine G (Colour Index No. 410), Chlorazol Black LF (Colour Index No. 582), and the following 5 dyestuffs described in "Farbstofftabellen" by Gustav Schultz, 1932, vol. 2, 7th edition, on the pages given in parenthesis following their names: Chlorazol Brown PB (p. 50), Diamine Brilliant Scarlet S (p. 68), Diamine Fast Blue FFG (p. 69) and 10 Diamine Green HS (p. 70).

Having described our invention what we desire to secure by Letters Patent is:

1. Process for the production from at least two types of cellulosic yarns having different affinities for cotton dyestuffs of textile products capable of being dyed a solid shade with said dyestuffs, which comprises introducing into the yarns having the greater affinity for said dyestuffs acetyl radicles in a proportion corresponding with 20 a weight increase of from 1.5 to 2.5% whereby their affinity is reduced to that of the yarns having the lowest affinity and then forming the products from the modified and unmodified yarns.

2. Textile products capable of being dyed a 25 solid shade with a cotton dyestuff and containing a purely cellulosic yarn and at least one type of modified cellulosic yarn containing an acetyl radicle in a proportion corresponding with a weight increase of from 1.5 to 2.5% whereby the 30 modified yarn has a degree of affinity for cotton dyestuffs equal to that possessed by the purely cellulosic yarn.

GEORGE HOLLAND ELLIS.  
ROBERT WIGHTON MONCRIEFF.